



US005154779A

# United States Patent [19]

Holcombe et al.

[11] Patent Number: 5,154,779

[45] Date of Patent: Oct. 13, 1992

[54] **METHOD OF NITRIDING, CARBURIZING, OR OXIDIZING REFRACTORY METAL ARTICLES USING MICROWAVES**

[75] Inventors: Cressie E. Holcombe, Knoxville; Norman L. Dykes, Oak Ridge; Terry N. Tiegs, Lenoir City, all of Tenn.

[73] Assignee: Martin Marietta Energy Systems, Inc., Oak Ridge, Tenn.

[21] Appl. No.: 837,096

[22] Filed: Feb. 18, 1992

## Related U.S. Application Data

[63] Continuation of Ser. No. 512,306, Apr. 20, 1990, abandoned.

[51] Int. Cl. 5 C21D 1/09; H05B 6/64

[52] U.S. Cl. 148/207; 148/218; 148/220; 148/224; 148/241; 204/157.43; 219/10.55 R; 427/585; 427/590

[58] Field of Search 148/207, 218, 220, 224, 148/241, 284; 204/157.15, 157.43, 157.46; 219/10.55 R, 10.55 D, 10.55 M; 427/46

## References Cited

### U.S. PATENT DOCUMENTS

- 2,739,907 3/1956 Nowak ..... 748/241  
 3,171,009 2/1965 Scheller et al. ..... 219/10.55 R  
 3,585,258 6/1971 Levinson ..... 219/10.55 R  
 4,057,702 11/1977 Lacombe-Allard ..... 219/10.55 A  
 4,100,386 7/1978 Bardet ..... 219/10.55 A  
 4,147,911 4/1979 Nishitani ..... 219/10.55 M  
 4,163,140 7/1979 Bardet ..... 219/10.55 B  
 4,189,629 2/1980 Kraze ..... 219/10.55 A  
 4,307,277 12/1981 Maeda et al. ..... 219/10.55 R  
 4,323,745 4/1982 Berggreen et al. ..... 219/10.55 F  
 4,529,856 7/1985 Meek et al. ..... 219/10.55 R  
 4,529,857 7/1985 Meek et al. ..... 219/10.55 M  
 4,559,429 12/1985 Holcombe ..... 219/10.55 M  
 4,565,669 1/1986 Collins et al. ..... 219/10.55 R  
 4,683,363 7/1987 Scovell ..... 219/10.55 A  
 4,743,340 5/1988 Wrenn, Jr. et al. ..... 162/224  
 4,757,172 7/1988 Palaith et al. ..... 219/10.55 M  
 4,764,102 8/1988 Takahashi ..... 219/10.55 R  
 4,767,902 8/1988 Palaith et al. ..... 219/10.55 M  
 4,771,153 9/1988 Fukushima et al. ..... 219/10.55 B  
 4,772,770 9/1988 Matsui et al. ..... 219/10.55 A  
 4,784,686 11/1988 Meek et al. ..... 219/10.55 R  
 4,806,718 2/1989 Seaborne et al. ..... 219/10.55 E  
 4,808,780 2/1989 Seaborne ..... 219/10.55 E  
 4,810,846 3/1989 Holcombe et al. ..... 219/10.55 R  
 4,880,578 11/1989 Holcombe et al. ..... 264/2 G

### FOREIGN PATENT DOCUMENTS

1202810 8/1970 United Kingdom ..... 148/241

## OTHER PUBLICATIONS

C. E. Holcombe and N. L. Dykes, "High-Temperature Microwave Sintering of Nonoxide Ceramics," *91st Annual Meeting of the American Ceramics Society*, Apr. 25, 1989.

C. E. Holcombe, T. T. Meek, and N. L. Dykes "Unusual Properties of Microwave-Sintered Yttria-2 wt. % Firconia," *J. Mat'l Sc. Letters*, 7, 881-884 (1988).

C. E. Holcombe, T. T. Meek, and N. L. Dykes "Enhanced Thermal Shock Properties of Y<sub>2</sub>O<sub>3</sub>-2 wt. % ZrO<sub>2</sub> Heated Using 2.45 GHz Radiation," *Mat. Res. Soc. Symp. proc.*, vol. 124, Apr. 5-8 (1988).

W. H. Sutton, "Microwave Processing of Ceramic Materials," *Ceramic Bulletin*, vol. 68, No. 2, 376-286 (1989).

C. E. Holcombe, "New Microwave Coupler Material", *Am. Ceram. Soc. Bulletin*, vol. 62, 1388 (1983).

J. A. Mangels, "Effect of Rate-Controlled Nitriding and Nitrogen Atmospheres on the Formation of Reaction-Bonded Si<sub>3</sub>N<sub>4</sub>," *Am. Ceram. Soc. Bull.*, 60, 613-617 (1981) Discusses Rate-Controlled Nitriding.

J. M. Blocher, Jr. "Nitrides", *High-Temperature Materials and Technology*, Chap. 11, 379-382 (1967) Discusses Nitrides of Transition Elements of the Third, Fourth, Fifth, and Sixth Groups of the Periodic Table.

*The Condensed Chemical Dictionary*, Van Nostrand Reinhold Company, Tenth Edition, 741, 887 (1981) Discusses Definitions of "Nonmetal" and Refractory.

R. I. Jaffee, D. J. Maykuth, and E. M. Sherwood, "Refractory Metals and Metalloids", *High-Temperature Materials and Technology*, Ch. 6, 152-154 (1967) Discusses Refractory Metals and Metalloids.

Primary Examiner—George Wyszomierski  
 Attorney, Agent, or Firm—Ivan L. Ericson; Preston H. Smirman

## ABSTRACT

A method of nitriding an article of refractory-nitride-forming metal or metalloids. A consolidated metal or metalloid article is placed inside a microwave oven and nitrogen containing gas is introduced into the microwave oven. The metal or metalloid article is heated to a temperature sufficient to react the metal or metalloid with the nitrogen by applying a microwave energy within the microwave oven. The metal or metalloid article is maintained at that temperature for a period of time sufficient to convert the article of metal or metalloid to an article of refractory nitride. In addition, a method of applying a coating, such as a coating of an oxide, a carbide, or a carbo-nitride, to an article of metal or metalloid by microwave heating.

42 Claims, No Drawings

## METHOD OF NITRIDING, CARBURIZING, OR OXIDIZING REFRACRY METAL ARTICLES USING MICROWAVES

This invention was made with Government support under Contract No. DE-AC05-84OR21400 awarded by the U.S. Department of Energy to Martin Marietta Energy Systems, Inc. and the Government has certain rights in this invention.

This application is a continuation of application Ser. No. 07/512,306, filed Apr. 20, 1990, now abandoned.

### FIELD OF THE INVENTION

This invention relates to a method of nitriding. More 15 particularly, this invention relates to a method of nitriding metal and metalloid articles.

### BACKGROUND OF THE INVENTION

The nitrides of many metals and metalloids have high 20 melting points and are resistant to oxidation. Currently, powders of these nitrides are consolidated into a body, then the body is hot-pressed or hot-isostatic-pressed at high temperatures and pressures into a dense body. Operations of this type require expensive equipment and usually long periods of time. Also, bodies are frequently in a highly-stressed state after this type of heating and pressing operation.

The object of the subject invention is to provide a method for nitriding refractory metal and metalloid 30 articles to form dense, crack-free bodies of metal or metalloid nitrides, composites of these nitrides, coatings of these nitrides, and nitrides of metal and metalloid articles having a density less than theoretical density.

### SUMMARY OF THE INVENTION

In accordance with one aspect of the present invention, a new and improved method of nitriding a refractory-nitride forming metal or metalloid article comprises the following steps:

Step 1. A consolidated metal or metalloid article having an intimately contacting enwrapping of a ceramic insulating material is provided within a microwave oven.

Step 2. A nitrogen containing atmosphere is introduced into the microwave oven.

Step 3. The metal or metalloid article is heated by microwave energy within the microwave oven containing the nitrogen containing atmosphere to a temperature sufficient to react the metal or metalloid with the nitrogen by applying a microwave energy within the microwave oven.

Step 4. The metal or metalloid article is maintained at the temperature for a period sufficient to convert the metal or metalloid to a metal nitride or a metalloid 55 nitride.

In accordance with another aspect of the present invention, a new and improved method of providing a nitride coating on a metal or metalloid article comprises the following steps:

Step 1. A consolidated metal or metalloid article having an intimately contacting enwrapping of a ceramic insulating material is provided within a microwave oven.

Step 2. A nitrogen containing atmosphere is introduced into the microwave oven.

Step 3. The metal or metalloid article is heated by microwave energy within the microwave oven contain-

ing the nitrogen containing atmosphere to a temperature sufficient to react the metal or metalloid with the nitrogen by applying a microwave energy within the microwave oven.

Step 4. The metal or metalloid article is maintained at the temperature for a period sufficient to form a coating of metal nitride or metalloid nitride on the article of metal or metalloid.

In accordance with another aspect of the present invention, a new and improved method of providing an oxide coating on a refractory-oxide-forming metal or metalloid article comprises the following steps:

Step 1. A consolidated refractory-oxide-forming metal or metalloid article having an intimately contacting enwrapping of a ceramic insulating material is provided within a microwave oven.

Step 2. An atmosphere containing oxygen is introduced into the microwave oven.

Step 3. The refractory-oxide-forming metal or metalloid article is heated by microwave energy within the microwave oven containing the atmosphere to a temperature sufficient to react the refractory-oxide-forming metal or metalloid with the oxygen contained in the atmosphere by applying a microwave energy within the microwave oven.

Step 4. The refractory-oxide-forming metal or metalloid article is maintained at the temperature for a period sufficient to form a coating of oxide on the article of the refractory-oxide-forming metal or metalloid.

In accordance with another aspect of the present invention, a new and improved method of providing a carbide coating on a refractory-carbide-forming metal or metalloid article comprises the following steps:

Step 1. A consolidated refractory-carbide-forming metal or metalloid article having an intimately contacting enwrapping of a ceramic insulating material is provided within a microwave oven.

Step 2. A carbon containing atmosphere is introduced into the microwave oven.

Step 3. The refractory-carbide-forming metal or metalloid article is heated by microwave energy within the microwave oven containing the carbon containing atmosphere to a temperature sufficient to react the refractory-carbide-forming metal or metalloid with the methane contained in the atmosphere by applying a microwave energy within the microwave oven.

Step 4. The refractory-carbide-forming metal or metalloid article is maintained at the temperature for a period sufficient to form a carbide coating on the article of the refractory-carbide-forming metal or metalloid.

In accordance with another aspect of the present invention, a new and improved method of providing a metal carbo-nitride coating on a refractory-“carbo”-nitride-forming metal or metalloid article comprises the following steps:

Step 1. A consolidated refractory-“carbo”-nitride-forming metal or metalloid article having an intimately contacting enwrapping of a ceramic insulating material is provided within a microwave oven.

Step 2. A carbon and nitrogen containing atmosphere is introduced into the microwave oven.

Step 3. The refractory-“carbo”-nitride-forming metal or metalloid article is heated by microwave energy within the microwave oven containing the carbon and nitrogen containing atmosphere to a temperature sufficient to react the refractory-“carbo”-nitride-forming metal or metalloid with the methane and nitrogen con-

tained in the atmosphere by applying a microwave energy within the microwave oven.

Step 4. The refractory-“carbo”-nitride-forming metal or metalloid article is maintained at the temperature for a period sufficient to form a carbo-nitride coating on the article of refractory-“carbo”-nitride-forming metal or metalloid.

#### DETAILED DESCRIPTION OF THE PREFERRED EMBODIMENTS

The new and improved method of the present invention for fabricating of refractory-nitride forming metal or metalloid dense articles, composites and coatings comprises the following operations (where refractory-nitride-forming “metal” refers to Ti, Zr, Hf, Nb, Ta, and Al; and where “metalloid” refers to refractory-nitride-forming nonmetals such as Si and B):

1) consolidating (i.e., pressed powder) at least one material selected from the group consisting of refractory metals, refractory metal nitrides, aluminum, silicon, and boron into a selected configuration;

2) surrounding the configuration with an intimately contacting enwrapping of a ceramic aggregate of granular material having an average particle size ranging from 2  $\mu\text{m}$  to +100 mesh and selected from the group consisting of alumina, calcia, magnesia, yttria, and silicon nitride in which the granular materials are electrical and thermal insulators and essentially noncouplers with microwaves to prevent electrical sparking and to provide thermal insulation for the configuration; and

3) heating the enwrapped configuration with microwaves in a nitrogen atmosphere or a nitrogen containing atmosphere such as  $\text{NH}_3$  or mixtures of  $\text{N}_2-\text{H}_2$ ,  $\text{NH}_3-\text{H}_2$ ,  $\text{N}_2-\text{Ar}$ , or  $\text{N}_2$ -inert gas to a desired temperature for conversion of any non-nitride portion in the enwrapped material to a nitride and densification of the formed nitrides.

#### EXAMPLE I

In a demonstration of the subject invention, a powder mixture containing 50 wt % niobium, 20 wt % tungsten and 30 wt % titanium nitride was pressed into a disc having a diameter and a thickness of 1 inch. The disc was surrounded with grit of yttria having a particle size ranging from 150 to 425 microns in an encasement of alumina brick that had been arranged in a microwave oven. The oven was equipped with a standard-energy (1.6 kW) and standard frequency (2.45 GHz) microwave unit.

In the heating operation, the disc was exposed to the maximum energy level of 1.6 kW for 100 minutes in an environment of flowing nitrogen. Then, the power switch on the oven was moved to the “off” position and the disc was cooled to ambient temperature in the flowing nitrogen. The cooled disc was removed from the arrangement in the oven and easily brushed free of the yttria granules.

The disc was visually examined for cracks, then the physical characteristics of the disc were determined.

The tests indicated that the disc was completely sintered and crack free. Standard mercury intrusion porosimetry techniques indicated a real density of 7.68 g/cc, an open porosity of 40% and a closed porosity of 4%.

Analyses indicated that the disc contained 53.5% of niobium nitride, 27.9% of titanium nitride and 18.6% of tungsten.

#### EXAMPLE II

In another demonstration of the subject invention, a powder mixture containing 50 wt % niobium, 20 wt % tungsten and 30 wt % titanium nitride was pressed into a disc having a diameter and thickness of 1 inch. The disc was surrounded in alumina grit having a particle size ranging from 150 to 425 microns in an encasement of alumina brick, except alumina grit was used instead of yttria granules. This arrangement was assembled in a microwave oven, and the metals contained in the disc were converted to a nitride of the metals and sintered as described in Example I.

The processed disc was visually examined for cracks, then the physical characteristics of the disc were determined. These tests indicated that the disc was completely sintered and crack-free. Standard mercury intrusion porosimetry techniques indicated a real density of 7.7 g/cc, an open porosity of 42% and a closed porosity of 4%. Analyses indicated that the disc contained 53 wt % of niobium nitride, 28 wt % titanium nitride and 19 wt % of tungsten.

#### EXAMPLE III

A powder mixture having a 99% purity and 325-mesh particles was pressed into a disc. The powder mixture contained 88.1 wt % elemental silicon, 9.5 wt % yttrium oxide and 2.4 wt % aluminum oxide. Also, the pressed disc had a diameter of 1 inch and a thickness of 0.5 inch. In preparation for the heating operation, the disc was surrounded in yttria grit with particle sizes ranging from 150 to 425 microns inside a case of alumina brick. This arrangement was assembled inside a microwave oven. The pressed disc was converted to a nitride composite and sintered by the procedure described in EXAMPLE I.

Visual examination indicated that the processed disc was free of cracks. The processed disc was designed to convert to a composition consisting of 92.5 wt % silicon nitride, 6.0 wt % yttrium oxide and 1.5 wt % aluminum oxide, with a theoretical density of 3.2 g/cc. Dimensional measurements indicated the density of the processed disc was 70% of the theoretical density.

Control of the temperatures (1400° to 1875° C.) and time period of exposure (10 to 100 minutes) is required to obtain full density. However, this experiment indicated that ceramic compositions with a silicon nitride base can be synthesized by the subject development.

#### EXAMPLE IV

A silicon powder consisting of greater than 99.95% purity was pressed into a cylindrical compact having approximate dimensions of 2 inches diameter and 1.75 inches in length. The sample was placed in a boron nitride crucible containing silicon nitride—2 wt % yttria powder having an average particle size of approximately 2  $\mu\text{m}$ . An alumina fiber board was placed around the crucible. This arrangement was placed in a microwave oven and the oven filled with nitrogen gas.

The compact temperature was monitored by a thermocouple and heated to 1400° C. oven for about 23 hr. The compact was converted to greater than 78% silicon nitride.

#### EXAMPLE V

A powder mixture consisting of 86.9 wt % silicon (>99.95%), 9.8 wt % yttria and 3.3 wt % alumina were blended together and pressed into a compact and

placed in a crucible as described in Example IV and the arrangement as described in Example IV was placed in the oven. The oven was filled with argon gas. The temperature of the compact was then raised to approximately 1000° C. Nitrogen was then flowed into the microwave furnace and the temperature raised to 1400° C. The total treating time in the microwave oven was about 24 hr. The compact was converted to greater than 75% silicon nitride.

Synthesis of silicon nitride by direct reaction of a silicon bar with nitrogen is known in the art. However, the use of powder and of microwave radiation for heating the compacted powder is believed to be new. It was not known that elemental silicon could be heated to a temperature sufficient for conversion to silicon nitride with microwave radiation.

#### EXAMPLE VI

A sample of -325 mesh powder of niobium-1 wt. % zirconium (Nb-1Zr) alloy was pressed into a disc having a diameter of 1 inch and a thickness of 0.5 inch. The disc was arranged in a microwave oven as described in EXAMPLE I, then exposed to the maximum energy level (1.6 kw) for 90 minutes in flowing argon. The environment of the furnace was changed from flowing argon to flowing nitrogen, then heated for 5 minutes in the nitrogen environment at the maximum energy level. The disc was cooled in the nitrogen environment and removed from the microwave oven.

Visual inspection indicated that the processed disc was free of cracks. Microscopic examination indicated that the surface of the processed disc was heavily nitrided and the interior of the processed disc metallic. A major portion of the surface nitride was identified as zirconium nitride and the composition beneath the nitride layer rapidly graded to a mixture of niobium and zirconium nitrides. The depth of the nitrided layer ranged from 1 to 2 mm.

It is believed that this method of coating surfaces could be used for coating surfaces with other compounds by using other reactive gases. For example, a surface could be coated with a refractory-oxide-forming metal or metalloid (where refractory-oxide-forming "metal" refers to Zr, Hf, Y, Sc and the rare earths, U, Th, Ti, Al, Cr; and "metalloid" refers to Si) by flowing oxygen (air) through the furnace. Similarly, a surface could be coated with a refractory-carbide-forming metal or metalloid (where refractory-carbide-forming "metal" refers to Ti, Zr, Hf, Nb, Ta, V, Cr, Mo, and W; and "metalloid" refers to Si and B) by flowing a carbon containing atmosphere such as methane, acetylene, butane, or mixtures thereof with argon, helium or hydrogen through the furnace. Also, surfaces could be coated with a refractory-carbo-nitride-forming metal or metalloid (where refractory-carbo-nitride-forming "metal" refers to Ti, Zr, Hf, Nb, and Ta; and "metalloid" refers to Si and B) by flowing a gas mixture of carbon containing gas such as methane, acetylene, butane or mixtures thereof with argon, helium, hydrogen or ammonia and nitrogen through the furnace. In a similar manner to these examples of forming nitrides, oxides and carbides, any mixed phase (such as the "carbo" nitrides illustrated) can be produced: oxycarbides and oxynitrides (i.e., Si-O-N) can be produced and used as mixed-metal phases (i.e., Si-Al-O-N). This coating technique could be very useful for coating items such as crucibles, drill bits and cutting tools with special coatings which have desired properties.

Refractory metal composites of refractory metals, silicon and aluminum are rapidly and efficiently converted to the nitride and densified in one operation. Also, poor microwave couplers, such as silicon nitride, can be relatively sintered from the microwave-coupling elemental silicon and formed into dense composites.

It is believed that the subject development is not limited to the preparation and densification of refractory nitrides. Other intermetallic materials such as the borides, carbides and silicides could be easily and efficiently prepared and densified with the subject method by simply selecting the proper materials and conditions.

In the subject invention, the production of silicon nitride in a gaseous reaction with the required heat provided by a flux of microwave radiation is believed to be a significant contribution to the state of the art. In other applications, materials such as intermetallics, composites and coatings can be produced by the subject method. The combination of materials in a composite can be varied by including reactive and nonreactive components in a composite. A hard ceramic coating of a material can be formed on drill bits, cutting tools, and crucibles; and surfaces of articles can be coated with intermetallic mixtures such as the carbo-nitrides.

Shown in Tables I, II, and III are the conditions of processing and the data obtained for numerous examples of compacts of elemental silicon powder (alone or with the typical additions of appropriate amounts of yttrium oxide [or yttrium nitrate] to yield 6 wt. %  $Y_2O_3$  and aluminum oxide [or aluminum nitrate] to yield 1.5%  $Al_2O_3$ ) being microwave-treated in nitrogen atmosphere to yield silicon nitride. For the microwave-reaction of silicon given in Tables I, II, and III, either a 1.6Kw fixed power or a 0 to 6Kw variable power, standard frequency (2.45 GHz) microwave applicator was used. With specimens up to several inches thickness and over four inches diameter, experiments showed that the nitridation was uniform; the nitride was distributed evenly throughout the compacts. Iron oxide (which is typically added as a nitriding catalyst in conventional nitriding operations) was tested in the standard 3 to 5 wt. % level; the nitriding was about the same with or without this iron oxide addition. This is very important, since the iron oxide addition lowers the melting point of the grain boundary mixed oxide phase, thus lowering the high-temperature utility of the resultant silicon nitride. Thus, microwaved silicon nitride has a decided advantage over conventional reaction-bonded silicon nitride since the microwaved material does not require the detrimental iron oxide addition.

Also, it has been shown quantitatively that microwave heating enhances the nitridation of silicon to produce reaction-bonded silicon nitride (or "RBSN"). With microwave nitridation, only about 12 hours is required at 1350° C. to get approximately 95% conversion of the silicon metal to silicon nitride; whereas, conventional nitridation would require around 160 hours to accomplish the same degree of conversion to silicon nitride. In other words, the microwave nitriding takes less than one-tenth the time of conventional nitriding.

RBSN is important since the dimension of the part essentially stays the same before and after nitriding, an unusual feature of the reactive nitriding of silicon—to yield a dimensionally constant part. The dimensions of the un-nitrided silicon compact are essentially the same as the dimensions of the nitrided part; thus, by this pro-

cess near-net-shape parts of silicon nitride can be produced.

The fact that microwave formation of silicon is so efficient may result from the enhanced reaction of the nitrogen at the grain-to-grain surfaces. Microwave energy is typically absorbed preferentially in the grain boundaries; micro-arcing may occur in the grain boundary regions. In any case, the nitriding of silicon is greatly enhanced. Silicon nitride (this is, completely nitrided silicon) is not a good microwave absorber. Thus, it is remarkable that silicon metal heats up readily

and also readily converts to silicon nitride when a nitrogen atmosphere is utilized.

The subject invention offers investigators of intermetallics a rapid and efficient method for preparation and densification of these materials and compositions of them.

While there has been shown and described what is at present considered the preferred embodiment of the invention, it will be obvious to those skilled in the art that various changes and modifications may be made therein without departing from the scope of the invention as defined by the appended claims.

TABLE I

| Sample # | Data on Microwave - Reacted Silicon Materials in Nitrogen Atmosphere |        |         |            |      |     | Ending Composition (wt. %) based on N <sub>2</sub> weight gain |         |       |         |            |         |
|----------|----------------------------------------------------------------------|--------|---------|------------|------|-----|----------------------------------------------------------------|---------|-------|---------|------------|---------|
|          | Starting Composition (wt. %)                                         |        |         | Iron Oxide |      |     | Silicon Nitride                                                | Silicon | Yttia | Alumina | Iron Oxide | Iron    |
|          | Silicon                                                              | Yttria | Alumina | Carbon     | Iron |     | Silicon                                                        | Silicon | Yttia | Alumina | Iron       | Silicon |
| 1        | 95.2                                                                 |        |         | 2.9        | 1.9  |     | 73.2                                                           | 20.3    |       |         | 2.0        | 4.5     |
| 2        | 88.1                                                                 | 9.5    | 2.4     |            |      |     | 79.8                                                           | 12.0    | 6.5   | 1.6     |            |         |
| 3        | 100.0                                                                |        |         |            |      |     | 76.9                                                           | 23.1    |       |         |            |         |
| 4        | 95.2                                                                 |        |         | 2.9        | 1.9  |     | 23.5                                                           | 68.1    |       |         | 2.6        | 5.7     |
| 5        | 90.6                                                                 | 8.0    |         |            |      | 1.4 | 37.6                                                           | 54.4    | 6.8   |         |            | 1.2     |
| 6        | 88.1                                                                 | 9.5    | 2.4     |            |      |     | 74.2                                                           | 17.5    | 6.7   | 1.7     |            |         |
| 7        | 88.1                                                                 | 9.5    | 2.4     |            |      |     | 71.0                                                           | 20.4    | 6.8   | 1.7     |            |         |
| 8        | 88.1                                                                 | 9.5    | 2.4     |            |      |     | 28.2                                                           | 61.2    | 8.4   | 2.1     |            |         |
| 9        | 88.1                                                                 | 9.5    | 2.4     |            |      |     | 29.4                                                           | 60.1    | 8.4   | 2.1     |            |         |
| 10       | 88.1                                                                 | 9.5    | 2.4     |            |      |     | 65.9                                                           | 25.3    | 7.0   | 1.7     |            |         |
| 11       | 44.05                                                                | 4.75   | 1.2     |            |      |     | 50.0                                                           | 89.1    | 6.2   | 3.8     | 1.0        |         |
| 12       | 95.2                                                                 |        |         | 2.9        | 1.9  |     |                                                                | 71.7    | 21.7  |         | 2.1        | 4.5     |
| 13       | 95.2                                                                 |        |         | 2.9        | 1.9  |     |                                                                | 67.5    | 25.8  |         | 2.1        | 4.6     |

TABLE II

| Microwaving Conditions, Using 6Kw, 2.45 GHz Processing Unit |                                                                  |                                       |                            |                                          |                      |                       |     |
|-------------------------------------------------------------|------------------------------------------------------------------|---------------------------------------|----------------------------|------------------------------------------|----------------------|-----------------------|-----|
| Sam- ple #                                                  | Specimen Dimensions<br>Inches (cm)<br>D = diameter<br>h = height | Initial Pellet Pressure<br>Conditions | Weights +<br>Initial/Final | Soak Temperature<br>T <sub>1</sub> (°C.) | T <sub>2</sub> (°C.) | Heat-up Time<br>(min) |     |
| 1                                                           | D = 7.0 (17.7)<br>h = 2.0 (5.0)                                  | Isostatic,<br>10,000 psi              | 1998.3                     | 2823.7                                   | 1200-<br>1400        |                       | ~30 |
| 2                                                           | D = 1.0 (2.5)<br>h = 0.67 (1.7)                                  | Unidirectional<br>4,000 psi           | 13.24                      | 19.44                                    | 1260-<br>1400        | 1500-<br>1530         | 5   |
| 3                                                           | D = 1.0 (2.5)<br>h = 0.25 (0.64)                                 | Unidirectional<br>4000 psi            | 3.57                       | 5.15                                     | 1260-<br>1400        | 1500-<br>1530         | 5   |
| 4                                                           | D = 1.4 (3.6)<br>h = 2.0 (5.0)                                   | Isostatic,<br>10,000 psi              | 90.68                      | 100.14                                   | 1235-<br>1370        | 1700                  | 20  |
| 5                                                           | D = 1.0 (2.5)<br>h = 0.63 (1.6)                                  | Unidirectional<br>4,000 psi           | 12.74                      | 14.99                                    | 1235-<br>1370        | 1700                  | 20  |
| 6                                                           | D = 1.0 (2.5)<br>h = 0.74 (1.9)                                  | Unidirectional<br>4,000 psi           | 15.00                      | 21.30                                    | 1380-<br>1400        |                       | 17  |
| 7                                                           | D = 1.0 (2.5)<br>h = 0.71 (1.8)                                  | Unidirectional<br>10,000 psi          | 17.65                      | 24.64                                    | 1300-<br>1400        |                       | 27  |
| 8                                                           | D = 1.0 (2.5)<br>h = 0.54 (1.4)                                  | Unidirectional<br>10,000 psi          | 13.44                      | 15.15                                    | 1435-<br>1470        | 1550-<br>1800         | 15  |
| 9                                                           | D = 1.0 (2.5)<br>h = 0.55 (1.7)                                  | Unidirectional<br>5,000 psi           | 13.69                      | 15.51                                    | 1435-<br>1470        | 1550-<br>1800         | 15  |
| 10                                                          | D = 1.0 (2.5)<br>h = 0.68 (1.7)                                  | Unidirectional<br>4,000 psi           | 13.92                      | 18.89                                    | 1250-<br>1350        |                       | 150 |
| 11                                                          | D = 1.0 (2.5)<br>h = 0.54 (1.4)                                  | Unidirectional<br>4,000 psi           | 11.51                      | 14.29                                    | 1275-<br>1400        |                       | 26  |
| 12                                                          | D = 1.0 (2.5)<br>h = 0.54 (1.4)                                  | Isostatic<br>10,000 psi               | 11.40                      | 15.97                                    | 1360-<br>1400        |                       | 54  |
| 13                                                          | D = 1.4 (3.6)<br>h = 3.5 (8.9)                                   | Isostatic<br>10,000 psi               | 140.37                     | 192.11                                   | 1300-<br>1400        | 1450-<br>1600         | 60  |

| Sam- ple # | Holding Time at T <sub>1</sub> (min) | Holding Time at T <sub>2</sub> (min) | Power Input T <sub>1</sub> (Kw) | Power Input T <sub>2</sub> (Kw) | "Casket" Packing Media Insulation | Final Specimen Density | % of Theoretical Density |
|------------|--------------------------------------|--------------------------------------|---------------------------------|---------------------------------|-----------------------------------|------------------------|--------------------------|
| 1          | 1395                                 |                                      | 3.5-6.0                         |                                 | Zirconia Bubbles and Fiber        | 2.29                   | 75                       |
| 2          | 160                                  | 60                                   | 0.5-3.0                         | 3.0-4.0                         | Zirconia Bubbles                  | 2.26                   | 70                       |
| 3          | 160                                  | 60                                   | 0.5-3.0                         | 3.0-4.0                         | Zirconia Bubbles                  | 1.59                   | 53                       |

TABLE II-continued

| Microwaving Conditions. Using 6Kw, 2.45 GHz Processing Unit |     |     |         |         |                      |      |    |
|-------------------------------------------------------------|-----|-----|---------|---------|----------------------|------|----|
| 4                                                           | 7   | 303 | 0.5     | 0.5-1.2 | Zirconia<br>Fiber    | 1.99 | 80 |
| 5                                                           | 7   | 303 | 0.5     | 0.5-1.2 | Zirconia<br>Fiber    | 2.21 | 76 |
| 6                                                           | 152 |     | 0.6-1.0 |         | Zirconia<br>Bubble   | 2.22 | 70 |
| 7                                                           | 180 |     | 0.5-1.4 |         | Zirconia<br>Bubble   | 2.68 | 85 |
| 8                                                           | 67  | 85  | 0.4-0.7 | 0.4-0.5 | Fused<br>Yttria Grit | 2.16 | 76 |
| 9                                                           | 67  | 85  | 0.4-0.7 | 0.4-0.5 | Fused<br>Yttria Grit | 1.81 | 64 |
| 10                                                          | 150 |     | 0.5-0.7 |         | Zirconia<br>Bubble   | 2.17 | 70 |
| 11                                                          | 84  |     | 2.5-4.0 |         | Zirconia<br>Bubble   | 2.04 | 63 |
| 12                                                          | 85  |     | 0.9-1.0 |         | Zirconia<br>Bubble   | 2.31 | 76 |
| 13                                                          | 24  | 249 | 0.4-2.2 | 1.8-5.0 | Zirconia<br>Bubble   | 2.16 | 72 |

TABLE III

| Sample No. | Percentage if all reacted | Reaction Based On: Initial wt. Final wt. | Reaction Based On: N <sub>2</sub> Pickup | Total N <sub>2</sub> Pickup if all reacted | Comments                                                                                                                                                            |
|------------|---------------------------|------------------------------------------|------------------------------------------|--------------------------------------------|---------------------------------------------------------------------------------------------------------------------------------------------------------------------|
| 1          | 88                        |                                          |                                          | 68                                         | Utilizes Iron Oxides as a possible nitriding promoter.                                                                                                              |
| 2          | 93                        |                                          |                                          | 80                                         |                                                                                                                                                                     |
| 3          | 87                        |                                          |                                          | 67                                         |                                                                                                                                                                     |
| 4          | 69                        |                                          |                                          | 17                                         | Utilizes Iron Oxides as a possible nitriding promoter.                                                                                                              |
| 5          | 73                        |                                          |                                          | 29                                         | Utilizes Iron Metal as a possible nitriding promoter.                                                                                                               |
| 6          | 90                        |                                          |                                          | 72                                         |                                                                                                                                                                     |
| 7          | 88                        |                                          |                                          | 68                                         |                                                                                                                                                                     |
| 8          | 71                        |                                          |                                          | 22                                         |                                                                                                                                                                     |
| 9          | 71                        |                                          |                                          | 23                                         |                                                                                                                                                                     |
| 10         | 86                        |                                          |                                          | 61                                         |                                                                                                                                                                     |
| 11         | 93                        |                                          |                                          | 73                                         | 50/50 Blend by weight of Pre-Reacted Silicon Nitride Powder and a Si/Y <sub>2</sub> O <sub>3</sub> /Al <sub>2</sub> O <sub>3</sub> mix of composition 88.1/9.5/2.4% |
| 12         | 87                        |                                          |                                          | 66                                         | Utilizes Iron Oxide as a possible nitriding promoter.                                                                                                               |
| 13         | 85                        |                                          |                                          | 61                                         | Utilizes Iron Oxide as a possible nitriding promoter. This sintered log was shown by microprobe to have a completely uniform distribution of nitrogen throughout.   |

What is claimed is:

1. A method of nitriding an article of refractory-nitride-forming metal or metalloid comprising the following steps:

Step 1) providing an article of metal or metalloid having an intimately contacting enwrapping of a ceramic insulating material within a microwave oven;

Step 2) introducing a nitrogen containing atmosphere within said microwave oven, said nitrogen containing atmosphere comprises gases selected from the group consisting of ammonia, nitrogen and mixtures thereof;

Step 3) heating said article of metal or metalloid in said nitrogen containing atmosphere within said microwave oven to a temperature sufficient to react with said article of metal or metalloid with said nitrogen by applying a microwave energy within said microwave oven; and

Step 4) maintaining said article of metal or metalloid at said temperature for a period of time sufficient to convert said article of metal or metalloid to an article or refractory nitride.

2. A method in accordance with claim 1 wherein said article comprises a metal selected from the group consisting of titanium, tantalum, hafnium, zirconium, nio-

rium and mixtures thereof or change said article comprises a metalloid selected from the group consisting of silicon, boron, and mixtures thereof.

3. A method in accordance with claim 2 wherein said article in Step 1 is silicon, said period of time in Step 4 is about 12 hours, said temperature in Step 3 is about 1350° C. in order to obtain approximately 95% conversion of silicon to silicon nitride.

4. A method in accordance with claim 1 wherein said article comprises materials selected from the group consisting of silicon, carbon, iron, and mixtures thereof, and said ceramic insulating material comprises materials selected from the group consisting of yttria, alumina, iron oxide, silicon nitride, and mixtures thereof.

5. A method in accordance with claim 1 wherein said microwave energy in Step 3 is generated by a 2.45 GHz microwave oven.

6. A method in accordance with claim 1 wherein in step 1 said article of metal or metalloid is enwrapped in a ceramic aggregate of granular material which further is contained in a refractory ceramic container, said granular material having an average particle size ranging from -4 to +100 mesh and being in intimate contact with said article of metal or metalloid.

7. A method in accordance with claim 1 wherein said temperature in Step 3 is greater than 1,000 degrees centigrade.

8. A method in accordance with claim 1 wherein said article of refractory nitride has a density up to and including 85% of theoretical density.

9. A method in accordance with claim 1 wherein said nitrogen containing atmosphere contains gases selected from the group consisting of ammonia, nitrogen and mixtures thereof and gases selected from the group 10 consisting of hydrogen, inert gases and mixtures thereof.

10. A method in accordance with claim 9 wherein said inert gases are selected from the group consisting of argon, helium and mixtures thereof.

11. A method of providing a metal nitride coating on an article of metal or metalloid comprising the following steps:

Step 1) providing an article of metal or metalloid 20 having an intimately contacting enwrapment of a ceramic insulating material within a microwave oven;

Step 2) introducing a nitrogen containing atmosphere 25 within said microwave oven, said nitrogen containing atmosphere comprises gases selected from the group consisting of ammonia, nitrogen and mixtures, thereof;

Step 3) heating said article of metal or metalloid in 30 said nitrogen containing atmosphere within said microwave oven to a temperature sufficient to react with said article of metal or metalloid with said nitrogen by applying a microwave energy within said microwave oven; and

Step 4) maintaining said article of metal or metalloid 35 at said temperature for a period of time sufficient to form a coating of nitride on said article of refractory metal or metalloid.

12. A method in accordance with claim 11 wherein said article comprises a metal selected from the group 40 consisting of titanium, tantalum, hafnium, zirconium, niobium and mixtures thereof or said article comprises a metalloid selected from the group consisting of silicon, boron, and mixtures thereof.

13. A method in accordance with claim 11 wherein said article comprises materials selected from the group 45 consisting of silicon, carbon, iron, and mixtures thereof, and said ceramic insulating material comprises materials selected from the group consisting of yttria, alumina, iron oxide, silicon nitride, and mixtures thereof.

14. A method in accordance with claim 11 wherein said microwave energy in Step 3 is generated by a 2.45 50 GHz microwave oven.

15. A method in accordance with claim 11 wherein in step 1 said article of metal or metalloid is enwrapped in a ceramic aggregate of granular material which further 55 is contained in a refractory ceramic container, said granular material having an average particle size ranging from -4 to +100 mesh and being in intimate contact with said article of metal or metalloid.

16. A method in accordance with claim 11, wherein 60 said temperature in Step 3 is greater than 1,000 degrees centigrade.

17. A method in accordance with claim 11 wherein said period of time in Step 4 is less than 150 hours.

18. A method in accordance with claim 11 wherein 65 said nitrogen containing atmosphere contains gases selected from the group consisting of ammonia, nitrogen and mixtures thereof and gases selected from the

group consisting of hydrogen, inert gases and mixtures thereof.

19. A method in accordance with claim 18 wherein said inert gases are selected from the group consisting of argon, helium and mixtures thereof.

20. A method of providing an oxide coating on an article of refractory metal or metalloid comprising the following steps:

Step 1) providing an article of metal or metalloid having an intimately contacting enwrapment of a ceramic insulating material within a microwave oven;

Step 2) introducing an oxygen containing atmosphere within said microwave oven, said oxygen containing atmosphere being comprised of air;

Step 3) heating said article of metal or metalloid in said atmosphere within said microwave oven to a temperature sufficient to react said oxygen in said atmosphere with said article of metal or metalloid by applying a microwave energy within said microwave oven; and

Step 4) maintaining said article of metal or metalloid at said temperature for a period of time sufficient to form a coating of oxide on said article of metal or metalloid.

21. A method in accordance with claim 20 wherein said article comprises a refractory metal selected from the group consisting of titanium, yttrium, scandium, lanthanum, cerium, praseodymium, neodymium, promethium, samarium, europium, gadolinium, terbium, dysprosium, holmium, erbium, thulium, ytterbium, lutetium, hafnium, aluminum, chromium, uranium, thorium, zirconium, and mixtures thereof or said article comprises silicon.

22. A method in accordance with claim 20 wherein said microwave energy in Step 3 is generated by a 2.45 GHz microwave oven.

23. A method in accordance with claim 20 wherein in step 1 said article of metal or metalloid is enwrapped in a ceramic aggregate of granular material which further is contained in a refractory ceramic container, said granular material having an average particle size ranging from -4 to +100 mesh and being in intimate contact with said article of metal or metalloid.

24. A method in accordance with claim 20 wherein said atmosphere in Step 2 is provided by a flow of air into said microwave oven.

25. A method of providing a carbide coating on an article of metal or metalloid comprising the following steps:

Step 1) providing an article of metal or metalloid having an intimately contacting enwrapment of a ceramic insulating material within a microwave oven;

Step 2) introducing a carbon containing atmosphere within said microwave oven, said carbon containing atmosphere comprises gases selected from the group consisting of methane, acetylene, butane and mixtures thereof;

Step 3) heating said article of metal or metalloid in said atmosphere within said microwave oven to a temperature sufficient to react said methane in said atmosphere with said article of metal or metalloid by applying a microwave energy with said microwave oven; and

Step 4) maintaining said article of metal or metalloid at said temperature for a period of time sufficient to

form a coating of carbide on said article of metal or metalloid.

26. A method in accordance with claim 25 wherein said article comprise a metal selected from the group consisting of titanium, tungsten, hafnium, tantalum, vanadium, chromium, molybdenum, zirconium, niobium and mixtures thereof or said article comprises a metalloid selected from the group consisting of silicon, boron, and mixtures thereof.

27. A method in accordance with claim 25 wherein said carbon containing atmosphere contains gases selected from the group consisting of methane, acetylene, butane and mixtures thereof and gases selected from the group consisting of hydrogen, inert gases and mixtures thereof.

28. A method in accordance with claim 27 wherein said inert gases are selected from the group consisting of argon, helium and mixtures thereof.

29. A method in accordance with claim 25 wherein said microwave energy in Step 3 is generated by a 2.45 GHz microwave oven.

30. A method in accordance with claim 25 wherein in step 1 said article of metal or metalloid is enwrapped in a ceramic aggregate of granular material which further is contained in a refractory ceramic container, said granular material having an average particle size ranging from -4 to +100 mesh and being in intimate contact with said article of metal or metalloid.

31. A method of providing a metal carbo-nitride coating on an article of metal or metalloid comprising the following steps:

Step 1) providing an article of metal or metalloid having an intimately contacting enwrapping of a ceramic insulating material within a microwave oven;

Step 2) introducing a carbon and nitrogen containing atmosphere within said microwave oven, said carbon containing atmosphere in said carbon and nitrogen containing atmosphere comprises gases selected from the group consisting of methene, acetylene, butane, and mixtures thereof, said nitrogen containing atmosphere in said carbon and nitrogen containing atmosphere comprises gases selected from the group consisting of nitrogen, ammonia and mixtures thereof.

Step 3) heating said article of metal or metalloid in said atmosphere within said microwave oven to a temperature sufficient to react said methane and nitrogen in said atmosphere with said article of metal or metalloid by applying a microwave energy within said microwave oven; and

Step 4) maintaining said article of metal or metalloid at said temperature for a period of time sufficient to form a coating of carbo-nitride on said article of metal or metalloid.

32. A method in accordance with claim 31 wherein said article comprises a metal selected from the group consisting of titanium, tantalum, hafnium, zirconium, niobium and mixtures thereof or said article comprises a metalloid selected from the group consisting of silicon, boron, and mixtures thereof.

33. A method in accordance with claim 31 wherein said carbon and nitrogen containing atmosphere contains gases selected from the group consisting of ammonia, nitrogen and mixtures thereof and gases selected from the group consisting of methane, acetylene, butane and mixtures thereof and gases selected from the group

consisting of hydrogen, inert gases and mixtures thereof.

34. A method in accordance with claim 33 wherein said inert gases are selected from the group consisting of argon, helium and mixtures thereof.

35. A method in accordance with claim 31 wherein said microwave energy in Step 3 is generated by a 2.45 GHz microwave oven.

36. A method in accordance with claim 31 wherein in step 1 said article of metal or metalloid is enwrapped in a ceramic aggregate of granular material which further is contained in a refractory ceramic container, said granular material having an average particle size range from -4 to +100 mesh and being in intimate contact with said article of metal or metalloid.

37. A method of nitriding an article of silicon comprising the following steps:

Step 1) pressing a powder mixture comprising 86.9 wt. % silicon, 9.8 wt. % yttria, and 3.3 wt. % alumina to form a pressed article, said silicon having a purity greater than 99.95%;

Step 2) enwrapping said pressed article in a silicon nitride-2 wt. % yttria powder having a particle size of about 2  $\mu\text{m}$  contained in a boron nitride crucible, said crucible being covered by an alumina fiber board and placed in a microwave oven;

Step 3) introducing an argon containing atmosphere within said microwave oven, said argon containing atmosphere being comprised of argon gas;

Step 4) heating said article of silicon to a temperature of about 1000° C. in said argon atmosphere by applying a microwave energy within said microwave oven;

Step 5) introducing a nitrogen containing atmosphere within said microwave oven, said nitrogen containing atmosphere comprises gases selected from the group consisting of ammonia, nitrogen and mixtures thereof;

Step 6) increasing said temperature of said article of silicon to about 1400° C. in said nitrogen atmosphere by applying a microwave energy within said microwave oven; and

Step 7) maintaining said article of silicon at said temperature of Step 6 for a period of time sufficient to convert greater than 75% of said article of silicon to an article of silicon nitride, said article of silicon being heated by microwave energy for a period of about 24 hours.

38. A method of nitriding an article of metal or metalloid composite comprising the following steps:

Step 1) providing an article of metal or metalloid composite having an intimately contacting enwrapping of a ceramic insulating material within a microwave oven;

Step 2) introducing a nitrogen containing atmosphere within said microwave oven, said nitrogen containing atmosphere comprises gases selected from the group consisting of ammonia, nitrogen and mixtures thereof;

Step 3) heating said article of metal or metalloid composite in said nitrogen containing atmosphere within said microwave oven to a temperature sufficient to react with said metal or metalloid composite with said nitrogen by applying a microwave energy within said microwave oven; and

Step 4) maintaining said article of metal or metalloid composite at said temperature for a period of time

15

sufficient to convert said article of metal or metalloid composite to an article of refractory nitride.

39. A method in accordance with claim 38 wherein said article comprises a metal selected from the group consisting of titanium, tantalum, hafnium, zirconium, niobium, aluminum, and mixtures thereof or said article comprises a metalloid selected from the group consisting of silicon, boron, and mixtures thereof.

40. A method in accordance with claim 38 wherein said microwave energy in Step 3 is generated by a 2.45 10 GHz microwave oven.

41. A method in accordance with claim 38 wherein in step 1 said article of metal or metalloid composite is

16

enwrapped in a ceramic aggregate of granule materials which further is contained in a refractory ceramic container, said granular material having an average particle size ranging from -4 to +100 mesh and being in intimate contact with said article of metal or metalloid composite.

42. A method in accordance with claim 38 wherein said nitrogen containing atmosphere contains gases selected from the group consisting of ammonia, nitrogen and mixtures thereof and gases selected from the group consisting of hydrogen, inert gases and mixtures thereof.

\* \* \* \* \*

15

20

25

30

35

40

45

50

55

60

65